

Sept. 20, 1932.

C. E. K. MEES

1,878,961

PHOTOGRAPHIC ELEMENT OVERCOATED WITH A SCREENING DYE

Filed April 28, 1930

Fig. 1.



Fig. 2.



## UNITED STATES PATENT OFFICE

CHARLES E. KENNETH MEES, OF ROCHESTER, NEW YORK, ASSIGNOR TO EASTMAN KODAK COMPANY, OF ROCHESTER, NEW YORK, A CORPORATION OF NEW YORK

## PHOTOGRAPHIC ELEMENT OVERCOATED WITH A SCREENING DYE

Application filed April 28, 1930. Serial No. 447,823.

This invention relates to a photographic element and particularly to one in which is used a screening or overcoating dye for color photographic purposes, and especially to the use of screening dyes for motion picture film employed in certain methods for taking color motion pictures.

In taking still or motion pictures in color with superimposed films or emulsions sensitized to different colors, it is desirable to interpose between certain of the light sensitive layers screening layers which prevent certain rays from affecting the underlying emulsion. For example, in a two color process, a green 15 sensitive film and a red sensitive film are used with their emulsion surfaces practically in contact, the picture exposure being made through the support side of the green sensitive film. The green sensitive emulsion is given a thin top coat of a green absorbing substance which prevents the green rays from affecting the red sensitive emulsion which has a certain sensitivity to green. This green absorbing substance must not diffuse into the 20 green sensitive layer to any marked extent. There are a number of commercial color motion picture processes which employ such red and green sensitive films face to face.

One object of the present invention is the 25 preparation of such non-diffusing screening layers for coating upon sensitive emulsions.

Another object is to provide such a screening layer which will not penetrate too far into the emulsion but will be confined to a 30 thin surface layer.

A further object is to provide a colored overcoating which does not desensitize the emulsion over which it is coated.

A still further object is to provide a screening layer which will wash out or fade suitably 35 in the processing baths, that is, the ordinary solutions used for developing and fixing the film, so that the film in question, which is a negative, may be readily printed to produce the positive.

Other objects and advantages will be apparent from the following specification. I do not limit myself to two color processes nor to the particular colors or dyes mentioned as 40 examples.

It is to be understood that I apply the dye to the photographic emulsion in the form of a very thin overcoating. By overcoating I mean applying a thin layer on top of the sensitive emulsion, as distinguished from bathing or dyeing as commonly understood. By the latter methods it is difficult to properly restrict the penetration of the dye. If the dye penetration could be restricted, bathing or dyeing would be satisfactory.

Reference will now be made to the accompanying drawing.

Fig. 1 is an enlarged section of a film embodying my invention.

Fig. 2 shows in section two films face to face 45 as employed in the method of color photography with which my invention may be used.

These figures and the following explanation will make clearer the character of the 50 product resulting from the invention, together with certain advantages in its use.

The drawing (Fig. 1) shows in greatly magnified cross-section the cellulosic support 3 with the sensitive emulsion layer 4 coated thereon, and a thin dye layer 5 on top of the emulsion penetrating a relatively short distance into the emulsion layer. The direction of the light is from the support side, as shown by the arrow. The dye layer may be considered as consisting of dyed particles of silver halide and of gelatin, the number of these particles (concentration) in a given area, being very high on the top surface, but becoming less and less with increasing depth. At a relatively short distance (a practically microscopic thickness) there are no longer any of these dyed particles.

In considering the screening action of these minute color filters, it must be remembered that they absorb light of the color to which the emulsion in which they lie is sensitive. Therefore, any dyed particles which may be in the lower portion of the dye layer, and toward the light, will screen off or absorb the light to which the particles behind them (toward the surface of the dye layer) are sensitive. It will, therefore, be seen that if the dye layer penetrates to considerable depth, a great many of the sensitive halide particles

of the emulsion will be screened off from the light which can act upon them, as there will be more of such particles with dyed screening particles between them and the light. 5 The result is that the dye layer reduces the effectiveness of its own emulsion layer and in effect the emulsion and dye layer screens itself. This result is detrimental and is avoided by the use of the method and materials I now propose.

The result and purposes I achieve are also to be distinguished from those obtained in the use of certain dyes (chiefly yellow) for the manufacture of so-called "self screening" 15 plates. In the latter case it is desired to screen every separate particle from the action of light of certain wave-lengths, usually blue, violet and ultra violet. Therefore it is desirable to have the dye penetrate as deeply as 20 possible or to permeate the whole emulsion layer. For this reason the dye is usually added to the emulsion before coating.

The class of dyes which I have found particularly advantageous for use as screening 25 dyes are those known in the photographic art as sensitizing dyes. They are ordinarily used to add to photographic emulsions to confer color sensitiveness on them. The dyes which I use are of two classes, known as the 30 acid sensitizing dyes and the basic sensitizing dyes. These dyes may be used either from alcoholic solutions or from water solutions. Slightly different results are obtained by the use of the two solvents, and some of the 35 dyes in particular work better one way than another, that is, some of the dyes of these classes, for example, do not give satisfactory results in water solutions only, while a few give better results from water.

40 I use the term dye in the same sense in which it is customarily used in this art, namely, to refer to the dye itself or to any of its salts having the same characteristic properties.

45 Examples of the acid sensitizing dyes are the following: mono-chlorfluorescein, di-chlorfluorescein, tetra-chlorfluorescein, mono-bromfluorescein, di-bromfluorescein, tetra-bromfluorescein (eosin), di-iodofluorescein 50 (erythrosin), tetra-iodofluorescein (erythrosin B), tetra-chlor-tetra-iodofluorescein (Rose Bengal), Phloxine, tetra-iodo-di-chlorfluorescein, and a number of others.

55 Examples of the basic sensitizing dyes are the rhodamines especially rhodamine 6-G, pinaflavol, pinaflavol p-toluene sulphonate, orthochrome T, pinaverdol, acridine orange, thiazole yellow, quinoline red, isocyanines, pseudo-cyanines, carbocyanines, oxy-carbo-60 cyanines, thiocarbocyanines, kryptocyanines, styryl pyridines and styrylquinolines.

The acid sensitizing dyes are usually employed in the form of their ammonium salts, on account of their superior solubility in alcohol and in water, and because they dry to a

smooth adherent surface. As an example of their use for dye overcoatings, a solution is made of the following formula (Formula 1) and this is applied by means of the usual coating apparatus or machinery in the form of a thin coating on top of the previously 70 coated and dried emulsions.

#### Formula I

| A                                 |     |          |
|-----------------------------------|-----|----------|
| Tetra-iodofluorescein             | 10  | grams 75 |
| Ammonia, $\frac{1}{4}$ strength * | 6.5 | cc.      |
| Denatured alcohol                 |     |          |
|                                   | 300 | cc.      |
| B                                 |     |          |
| Fluorescein                       | 40  | grams    |
| Ammonia, $\frac{1}{4}$ strength   | 60  | cc.      |
| Denatured alcohol                 | 700 | cc.      |

\* This quarter strength ammonia solution is prepared from the ordinary commercial 28% ammonia by diluting to four times its volume. Mix A and B. Dilute for coating. (It is usually best to dilute the above total formula as mixed to something like  $\frac{1}{4}$  of its strength, that is, the above mixture of A and B is diluted with about two liters of alcohol—denatured.)

An example of a basic sensitizing dye used 85 in alcoholic solution is the following:

#### Formula II

|                                 |       |       |
|---------------------------------|-------|-------|
| Rhodamine 6-G                   | 8     | grams |
| Pinaflavol p-toluene sulphonate | 32    | grams |
| Denatured alcohol               | 1,000 | cc.   |

Although the alcohol used in this formula contains a small amount of water, it is desirable to add a little more water to increase the ease of spreading of the solution. Formula II is one which washes out entirely after 95 processing.

An example of a sensitizing dye applied from a water solution is the following:

#### Formula III

|                                    |          |          |
|------------------------------------|----------|----------|
| 1:2 diethyl 3:4 benzo thio isocya- | 8        | grams    |
| nine iodide                        | 1:10,000 | in water |

Where it is permissible to use water solutions, it is generally found that the sensitizing effect is increased, that is, the dyes not only perform the screening function but also 105 tend to increase the color sensitiveness of the emulsion. It is possible to use water with most of the dyes which tend to form colloidal aggregates, these dyes usually consisting of very large molecules (chemically speaking). 110

On the other hand, alcohol has other advantages in that it prevents swelling of the gelatin during coating and permits rapid drying, both of which result in less penetration of the dye into the emulsion.

Fig. 2 shows two films face to face, one of them overcoated by my invention, as they would ordinarily be employed in multicolor motion picture processes of the type described in the United States patent to Ives 1,320,760, granted November 4, 1910 and the British patents to Buchanan, 12,469 of 1914 and Battistini, 873 of 1915. Film 1 is the green sensitive component already described and Film 2 comprises a support 6 with a very fast red sensitive emulsion 7 which is in intimate contact with the emulsion of Film 1. Exposure is made through the support of Film 1 as shown by the arrow, the dye acting as a screen for the emulsion 7.

Color screen surface coatings made with the dyes mentioned above, and in the manner indicated, have, in general, several advantages over those made with other dyes heretofore used for the purpose. (1) They penetrate the emulsion to a minimum extent, providing a thin surface dyed layer; (2) They do not fog or desensitize. In some cases, particularly where the dyes are used in water solutions, the sensitiveness is actually enhanced by the dye due to its sensitizing action. (3) They are easily removed or changed to such tints as are not objectionable.

10 I consider as included in my invention all modifications and equivalents coming within the scope of the appended claims.

15 What I claim is:

1. A photographic element comprising a support, a sensitized layer thereon, and a 20 very thin layer of light restraining dye of a sensitizing type applied directly to the outer surface of the emulsion layer but not penetrating substantially into said layer, said dye being selected from the group consisting of 25 the iso-cyanines, pseudo-cyanines, carbo-cyanines, oxycarbo-cyanines, thio-carbo-cyanines, krypto-cyanines, styryl-pyridines, styryl-quinolines and the acid dyes of the fluorescein series.

30 2. A phonographic element comprising a support, a sensitized layer thereon, and a very thin layer of light restraining dye of a sensitizing type applied directly to the outer surface of the emulsion layer but not penetrating substantially into said layer, said dye being an ammonium salt of a dye selected from the group consisting of the iso-cyanines, pseudo-cyanines, carbo-cyanines, oxycarbo-cyanines, thiocarbo-cyanines, krypto-cyanines, styryl-pyridines, styryl-quinolines and the acid dyes of the fluorescein series.

35 3. The method of overcoating a photographic emulsion with a dye which comprises applying to the surface a very thin coat of 40 a solution containing alcohol and a sensitizing dye selected from the group consisting of the iso-cyanines, pseudo-cyanines, carbo-cyanines, oxycarbo-cyanines, thio-carbo-cyanines, krypto-cyanines, styryl-pyridines, the 45 styryl-quinolines, and the acid dyes of the fluorescein series.

50 Signed at Rochester, New York this 22nd day of April, 1930.

CHARLES E. KENNETH MEES.